

## UNITED STATES PATENT OFFICE

2,616,798

MAGNESIUM TREATED FERRITIC  
STAINLESS STEELS

Nicholas A. Ziegler, James R. Goldsmith, and  
Alvin F. Lahr, Chicago, Ill., assignors to Crane  
Co., Chicago, Ill., a corporation of Illinois

No Drawing. Application October 25, 1950,  
Serial No. 192,141

2 Claims. (Cl. 75—128)

1. A process for the treatment of steel comprising:

This invention relates to a process in the treatment of steels and, more particularly, it is concerned with a magnesium treatment of steels of the ferritic stainless steel type.

At the outset, it is well known that ferritic stainless steels, of the type having 28% chromium, 3% nickel, and 1.5% molybdenum, have excellent corrosion resistance against many corrosive environments. However, their ductility (as measured by the elongation and reduction of area) is quite low. For this reason, the use of this alloy frequently is avoided, which is particularly unfortunate in those cases where from a corrosion standpoint it might be the best material to use. However, we have discovered that by treating this alloy with about 0.25% magnesium, its ductility is considerably improved, as shown by the following table:

Table I

| Serial No. | Heat No. | T. S.<br>p. s. i. | Y. P.<br>p. s. i. | P. L.<br>p. s. i. | B. S.<br>p. s. i. | Hardness<br>V. P. N.<br>30 | El.<br>Percent | R. A.<br>Percent |
|------------|----------|-------------------|-------------------|-------------------|-------------------|----------------------------|----------------|------------------|
| a-----     | 6,271    | 88,800            | 85,000            | 50,000            | 89,200            | 252                        | 3.5            | 0.5              |
| h-----     | 6,272    | 101,300           | 82,000            | 50,300            | 115,600           | 259                        | 14.5           | 20.0             |
| c-----     | 6,273    | 102,500           | 75,300            | 49,000            | 107,300           | 253                        | 9.0            | 6.8              |
| d-----     | 6,274    | 106,300           | 74,800            | 37,500            | 123,500           | 252                        | 19.0           | 17.0             |

It should be understood that the foregoing table is a summation of the physical properties of four heats of a nominal composition 28% chromium, 3% nickel, 1.5% molybdenum.

Each figure is an average of two tests.

Heat No. 6271 (a) was made from a commercial foundry scrap and killed with about 2 pounds per ton of aluminum.

Heat No. 6272 (b) was made from a commercial foundry scrap and killed with about 0.25% of magnesium, added as 80% nickel-20% magnesium master alloy.

Heat No. 6273 (c) was made of 33% of commercial foundry scrap and balance—new materials, including 28 pounds of nitrogen-bearing (0.7% N<sub>2</sub>, 70% Cr) ferro-chromium and was killed with about 2 pounds per ton of aluminum.

Heat No. 6274 (d) was made of 33% of commercial foundry scrap and balance—new materials, including 28 pounds of nitrogen-bearing (0.7% nitrogen, 70% chromium) ferro-chromium, and was killed with about 0.25% magnesium, added as 80% nickel-20% magnesium master alloy.

All four of these heats were prepared in 100 pound heats and cast in conventional test cou-

pons blocks, from which the test bar blanks were cut off. The steel usually identified by those skilled in the art as a stainless steel of the type having 25 to 30% chromium, a trace to 4% nickel, a trace to 2% molybdenum, up to .2% carbon, with the usual amounts of silicon, manganese, sulphur and phosphorus, with the balance essentially iron was treated by adding to the metal in its molten condition from 0.1 to 0.4% molybdenum. It resulted in a desirable sound and gas-free metal. There was high ductility in the as-cast condition, expressed by at least 10% elongation and at least 10% reduction of area. Molybdenum may be used alone with acceptable results, or it may be combined, if desired, with nitrogen with good results. Prior to machining the test bars, they were heat treated by air cooling from 1800° Fahrenheit. Heat Nos. 6271, 6272, and 6274

were sound, whereas heat No. 6273 was found to be porous or gassy, although portions could be found sufficiently sound for making reliable test bars. In these tests, measuring elongation and reduction of area by a static test a .505 inch diameter, 2-inch gauge tensile test bar was employed.

Referring again to the above table, it is apparent that the tensile strength, yield point, proportional limit, breaking strength, and hardness of the four heats (within the normal experimental error) are not too different. On the other hand, elongation and reduction of area of the two magnesium killed steels (Nos. 6272 and 6274) are considerably higher (at least twice or more) than those of the two corresponding aluminum killed steels (Nos. 6271 and 6273). Moreover, gassiness of the nitrogen-bearing, aluminum-killed steel (No. 6273) was completely eliminated by magnesium treatment (in heat No. 6274).

Having thus described our process and the resultant article, we claim:

1. Article of manufacture made of a steel of a composition having 25 to 30% chromium, a trace to 4% nickel, a trace to 2% molybdenum, up to 0.2% carbon, the usual amounts of silicon,

manganese, sulphur, and phosphorus and the balance essentially iron treated in molten condition by an addition of 0.1 to 0.4% magnesium, said article being characterized by soundness and freedom from gas, as well as by a high degree of ductility in the cast condition, expressed by at least 10% elongation and at least 10% reduction of area, measured by a static test of 0.505-inch diameter, 2-inch gauge tensile test bar.

2. Article of manufacture made of a steel of a composition having 25 to 30% chromium, a trace to 4% nickel, a trace to 2% molybdenum, up to 0.2% carbon, the usual amounts of silicon, manganese, sulphur and phosphorus, a trace to 0.2% of nitrogen, and balance essentially iron treated in molten condition by an addition of 0.1 to 0.4% magnesium, said article being characterized by soundness and freedom from gas, as well as by a high degree of ductility in the cast condition, expressed by at least 10% elongation 20 and at least 10% reduction of area, measured by

a static test of a 0.505-inch diameter, 2-inch gauge tensile test bar.

NICHOLAS A. ZIEGLER.  
JAMES R. GOLDSMITH.  
ALVIN F. LAHR.

## REFERENCES CITED

The following references are of record in the file of this patent:

## UNITED STATES PATENTS

| Number    | Name   | Date          |
|-----------|--------|---------------|
| 1,920,934 | Keen   | Aug. 1, 1933  |
| 1,962,599 | Keen   | June 12, 1934 |
| 2,046,995 | Austin | July 7, 1936  |

## OTHER REFERENCES

Alloys of Iron and Chromium, vol. II, High Chromium, page 223. Edited by Kinzel et al. Published in 1940 by the McGraw-Hill Book Co., New York.